# EUROPEAN PATENT SPECIFICATION

(11) **EP 1 359 240 B1**
(45) Date of publication and mention of the grant of the patent: **04.04.2007**
(21) Application number: 03008859.5
(22) Date of filing: 28.04.2003
(51) Int. Cl.: D04H 1/42, D04H 1/54, D04H 1/58, D04H 3/12, D04H 3/14, D04H 5/06, D01F 8/06, D01F 8/10, D01F 8/12, D01F 8/14

(54) **IMPROVED BINDER FIBER AND NONWOVEN WEB COMPRISING BINDER FIBER AND ABSORBENT**
VERBESSERTE BINDEFASERN UND VLIESSTOFF MIT BINDEFASERN UND ABSORBIERENDEM MATERIAL
FIBRE DE LIAGE AMELIOREE ET NONTISSE COMPRENANT DES FIBRES DE LIAGE ET UN ABSORBANT

(30) Priority: 02.05.2002 US 137141
(43) Date of publication of application: 05.11.2003
(73) Proprietor: INVISTA Technologies S.à.r.l., 8001 Zürich (CH)
(72) Inventor: Lin, Tingdong, Mooresville, North Carolina 28217 (US)
(74) Representative: Zounek, Nikolai

(56) References cited:
- EP-A- 0 198 173
- WO-A-00/29655
- WO-A-00/29658
- WO-A-98/21279
- WO-A-99/46327
- US-A- 4 340 513
- US-A- 5 288 791
- US-A- 5 372 885
- US-A- 5 981 410
- US-B1- 6 190 768

## Description

### BACKGROUND OF THE INVENTION

### 1. Field of the Invention

The present invention relates to an improved binder fiber comprising the combination of a low-melt polyethylene base and a tackifier comprised from 1 to 5 % by weight of said low melt polyethylene base, said low melt polyethylene base is low melt fiber, the low melting portion of bicomponent fiber, or both.

The present invention relates to dry laid and wet laid nonwoven webs useful in diapers, incontinent pads, sanitary napkins, and other absorbent pads for liquids. In particular, these pads usually comprise binder and wood pulp or other absorbent material. Making suitable nonwoven webs for these uses requires good adhesion between the binder and the absorbent material. More specifically, the present invention relates to a nonwoven web comprising binder fiber and absorbent. Tackifiers include rosin, rosin esters, and terpene based, piperylene based, and hydrocarbon based compounds. Optionally, the binder with tackifier may also contain an adhesion promoter, usually grafted polyolefins, and an enhancement agent, usually inactive inorganic compounds in powder form.

### 2. Prior Art

Nonwoven webs particularly in the form of disposal absorbent articles such as disposable diapers, have had much success in the marketplace. However, there is always a need to improve these products and particularly in terms of their adhesion such that they do not fall apart during manufacturing, processing into articles, and during use. Prior to the present invention, it was known to form existing nonwovens from absorbent (wood pulp and optionally up to 25% by weight super absorbent polymer, SAP), and a binder such as a bicomponent fiber or a low melt polymer fiber. These existing compositions contained approximately 10% binder and approximately 80 to 90% by weight absorbent.

These nonwoven webs were first created by mixing the wood pulp (and optionally SAP) with the binder. This composition was then introduced into a heating zone, such that the lower melt material of the polymer, or the lower melting material of the bicomponent fiber would melt and coat at least a portion of most of the wood pulp fibers (and any optional SAP). The composition was then introduced into a cooling zone where the lower melting binder material would solidify thereby binding the wood pulp (and optional SAP) into a unitary web structure.

Optionally, other fibers may be introduced such as other synthetic fibers or natural fibers to achieve other desired characteristics such as low density, high loft, compression resistance, and fluid uptake rate.

U.S. Patent 5,981,410 to Hansen, et al. discloses bicomponent fibers blended with cellulose fibers such as pulp fibers or cotton fibers to create a nonwoven web useful in disposable diapers, for example.

U.S. Patent 5,994,244 to Fujiwara, et al. discloses a nonwoven web comprised of cellulose type fibers such as fluff pulp and low melt fibers useful in producing disposable diapers, among other things. It also discloses the addition of inorganic particle (e.g. TiO₂) to the ethylene-acrylic ester-maleic anhydride sheath bicomponent spunbond filament. The particles reduce the adhesion of the filaments during spinning and give a more uniform web.

Suitable bicomponent fibers can be found in U.S. Patent 4,950,541 to Tabor, et al. and U.S. Patent 5,372,885 to Tabor, et al., both of which are hereby incorporated by reference. These patents disclose the use of a low melt maleic acid or maleic anhydride grafted polyethylene.

U.S. Patent 5,126,201 to Shiba et al. discloses the addition of TiO₂ in both the core and sheath of bicomponent binder fibers to improve the cutting efficiency of nonwoven webs. The amount of TiO₂ in the core is >1.5%, preferably there is no TiO₂ in the sheath, since TiO₂ in the sheath reduces adhesion.

U.S. Patent 5,288,791 discloses an elastic nonwoven web formed from elastic fibers composed of a blend of styrene-poly(ethylene-propylene)-styrene elastomeric copolymers, styrene-poly(ethylene-butylene)-styrene elastomeric copolymers, or a mixture thereof, and a tackifying resin. The elastic nonwoven web has a stress relaxation of less than 30 percent. The can include a polyolefine and an extending oil to improve the processing or bonding characteristics of the polystyrene web. The elastic fibers are not binder fibers.

WO 00/29655 describes a nonwoven web composite formed from thermoplastic bicomponent filaments having adhesive properties and a component selected from other fibers and particles. After the bicomponent filaments are combined with the other fibers and/or particles, the adhesive properties of the bicomponent filaments result in a web having improved ability to entrap and contain the other fibers and/or particles within the web.

U.S. Patent 6 190 768 discloses bicomponent fibers and a tackifier. The bicomponent fibers have substantially random ethylene/styrene interpolymer as the core and a second polymer as the sheath. The melt temperatures of the core and the sheath are approximately the same so that the bicomponent fibers have neither a low nor a high melting portion. Japanese Patent JP 02-169718 to Matsuo et al. discloses polyolefin sheath/polyester core bicomponent fibers, the sheath containing 0.3-10% of inorganic particles (preferably TiO₂) to obtain a better softness and opacity of the web. This patent teaches that the addition of inorganic particles reduce the nonwoven strength.

### SUMMARY OF THE INVENTION

As stated previously, there is still a need in the art to improve the adhesion of these nonwoven webs. The present invention is an improvement over these existing nonwoven web products. In particular, the present invention improves the adhesion by employing a tackifier.

According to the invention an improved binder fiber comprises the combination of a low melt polyethylene base and a tackifier, comprised from I to 5 % by weight of said low melt polyethylene base, said low melt polyethylene base is a low melt fiber, the low melting portion of a bicomponent fiber, or both, wherein a nonwoven web made from such binder fiber has a bonding index at least 13,8% greater than a web containing said binder fiber without tackifier.

The present invention relates to either bicomponent fiber or low melt polymer fiber and a nonwoven web containing one of these fibers, and tackifier thereby producing a binder fiber respect, a web with improved adhesion. The bicomponent fiber contains a high melting portion and a low melting portion, with the low melting portion containing tackifier. If low melt fiber (instead of bicomponent fiber) was employed it likewise contains tackifier. Tackifiers include rosin, rosin esters, and terpene based, piperylene based, and hydrocarbon compounds.The tackifier is believed to act as an adhesion promoting agent better binding the absorbent material together into a unitary web. The low melt polymer fiber or the low melting portion of the bicomponent fiber is defined as " low melt base".

The present invention comprises a binder fiber containing tackifier. The binding fiber may be a bicomponent fiber for a typical low melt polymer fiber. The low melt base contains the tackifier. The finer fiber containing tackifier may optionally contain an adhesion promoter and an enhancement agent.

The web of the present invention comprises binder fiber containing tackifier and an absorbent. The absorbent may be synthetic or natural.

In the broadest sense, the present invention also comprises a web comprising from about 5 to about 25% by weight binder fiber and from about 75 to 95% by weight absorbent. The absorbent may be a natural absorbent or a super absorbent polymer or a combination of these.

### DESCRIPTION OF THE PREFERRED EMBODIMENTS

Suitable absorbents are natural or synthetic absorbents. Synthetic absorbents are primarily known as super absorbent polymers (SAP). The absorbents comprise 75 - 95 % by weight of the web. Natural absorbents are hydrophilic materials such as cellulosic fibers, wood pulp fluff, cotton, cotton linters, and regenerated cellulose fibers such as rayon, or a mixture of these. Preferred is wood pulp fluff, which is both inexpensive and readily available.

Absorbent pads employing natural absorbents may not provide adequate fluid intake for all circumstances. Also natural absorbents are very bulky. Accordingly, many absorbent pads employ SAP in relatively low quantities. This is because the cost of SAP is much higher than the cost of natural absorbents. Replacing some of the natural absorbents with SAP can reduce the overall bulk of the pad and/or provide superior fluid intake.

As used herein, the term "super absorbent polymer" or "SAP" refers to a water-swellable, generally water-insoluble material capable of absorbing at least about 10, desirably about 20, and preferably about 50 times or more its weight in water. The super absorbent polymer may be formed from organic material, which may include natural materials such as agar, pectin, and guar gum, as well as synthetic materials such as synthetic hydrogel polymers. Synthetic hydrogel polymers include, for example, carboxymethyl cellulose, alkali metal salts of polyacrylic acid, polyacrylamides, polyvinyl alcohol, ethylene maleic anhydride copolymers, polyvinyl ethers, hydroxypropyl cellulose, polyvinyl morpholinone, polymers and copolymers of vinyl sulfonic acid, polyacrylates, polyacrylamides, polyvinyl pyridine, and the like. Other suitable polymers include hydrolyzed acrylonitrile grafted starch, acrylic acid grafted starch, and isobutylene maleic anhydride copolymers and mixtures thereof. The hydrogel polymers are preferably lightly crosslinked to render the materials substantially water insoluble. Crosslinking may, for example, be by irradiation or covalent, ionic, van der Waals, or hydrogen bonding. Suitable materials are available from various commercial vendors such as the Dow Chemical Company, Allied Colloid, Inc., and Stockhausen, Inc. The super absorbent polymer may be in the form of particles, flakes, fibers, rods, films or any of a number of geometric forms.

The binder fibers of the present invention can either be in the form of a low melt fiber, or a bicomponent fiber. The low melting portion of the bicomponent fiber would comprise the same material as the low melt fiber. The preferred binder fiber of the present invention is the bicomponent. Binder fibers have an average length of from about 3 to about 75 mm. Binder fibers having a denier of between 1 and 10 are preferred. Suitable polyethylene may be high density polyethylene (HDPE), medium density polyethylene (MDPE), low density polyethylene (LDPE), linear low density polyethylene (LLDPE), ultra low density polyethylene (ULDPE); or a mixture of these. These polyolefins may be produced with either Ziegler-Natta or metallocene catalysts.

Bicomponent fibers can be of the type in which the low melting portion is adjacent to the high melting portion such as a side-by-side configuration, or a sheath-core configuration where the sheath is the low melting component and the core is the high melting component. The high melting portion may be selected from the class of polyolefins, such as polyethylene, polypropylene, and polybutylene; polyesters such as polyethylene terephthalate (PET), polybutylene terephthalate, polyethylene naphthalate, and the like; polyamides such as nylon 6, nylon 66; polyacrylates such as polymethacrylate, polymethylmethacrylate, and the like; as well as mixtures and copolymers of these. The low melting portion, in a suitable bicomponent fiber melts at a temperature of at least about 5°C lower than said high melting portion.

Suitable bicomponent fibers have a low melting portion that comprises from about 5 to about 75% by weight of the bicomponent fiber, with the remainder being the high melting portion. If, for example, a 50-50 bicomponent fiber is employed as the binder fiber, the 50% by weight low melting portion is low melt base polyolefin with less than about 40% by weight tackifier (with or without an adhesion promoter or enhancement agent, or a mixture thereof), and the 50% by weight high melting portion could be PET.

Ignoring other components for a moment, suitable bicomponent fibers are polyethylene/polypropylene; polyethylene/polyester (especially polyethylene terephthalate); polyethylene/nylon, as well as mixtures of these. Preferably polyethylene/polyester fibers, such as LLDPE/PET or polyethylene/polypropylene, such as LLDPE/PP are used. When both the low melting portion and the high melting portion of the bicomponent fiber contains polyolefins, the high melting polyolefin must have a melting point at least about 5 ° C higher than the low melting polyethylene.

Tackifiers include rosin, rosin esters, and terpene based, piperylene based, and hydrocarbon based compounds. Commercially available rosin based tackifiers are known as Foral 85 made by Hercules, Inc.; Permalyn 2085 made by Eastman Chemicals; or Escorez 5400 made by Mobil Exxon Chemical. Commercially available terpene based tackifiers are Zonarez, Zonatac and Nirez from Arizona Chemical Company. Commercially available piperylene based tackifiers are Picotac and Hercotac available from Hercules, Inc. A commercially available hydrocarbon based tackifier is Escorez 5400 from ExxonMobil. The preferred tackifier is rosin ester, and most preferred is a glycerin ester of tall oil rosin. The tackifier preferably comprises from about 0.1 to about 40% by weight of the low melt base, and preferably 0.5 to 10%, and most preferably 1 to 5 %.

The adhesion promoters, such as polyolefins grafted with maleic acidormaleic anhydride (MAH), both of which convert to succinic acid or succinic anhydride upon grafting to the polyolefin, can be optionally used in addition to the tackifier. The preferred incorporated MAH graft level is 10% by weight (by titration). Also, ethylene-acrylic copolymers, and a combination of this with the grafted polyolefins mentioned are suitable adhesion promoters. Commercially available maleic anhydride grafted polyethylene are known as ASPUN resins from Dow Chemical. Commercially available ethylene-acrylic copolymers are Bynel 2022, Bynol 21E533 and Fusabond MC 190D from DuPont, and the Escor acid terpolymers from ExxonMobil. The ethylene-acrylic copolymer comprises from about 1 to about 20% by weight based on the weight of the low melt base, and preferably from 5 to 15% by weight. The amount of grafted polyolefin adhesion promoter is such that the weight of incorporated maleic acid or maleic anhydride comprises from about 0.05% to about 2% by weight, and preferably from 0.1 to 1.5% based on the weight of the low melt base.

Enhancement agents can be optionally used in addition to the tackifier and the optional adhesion promoter. The enhancement agent can comprise any of titanium dioxide, talc, silica, alum, calcium carbonate, calcium oxide, magnesium and other oxides; titanium dioxide being preferred. The enhancement agent is employed in the polymer in an amount from about 0.1 to about 1% based on the weight of the low melt base. The particle size, in order to achieve good dispersion within the polymer and good spinnability is in the range of about 0.04 to about 5 microns, and preferably in the range of 0.05 to 2 micron.

Once the low melt base with tackifier and any adhesion promoter and any enhancement agent is produced, preferably by blending master batches to the low melt base, it is melt spun into fiber as is known in the art.

Webs of the present invention can be made by either dry laid or wet laid processes. Dry laid webs are made by the airlay, carding, garneting, or random carding processes. Airlaid webs are created by introducing the fibers into an air current, which uniformly mixes the fibers and then deposits them on a screen surface. The carding process separates tufts into individual fibers by combing or raking the fibers into a parallel alignment. Garneting is similar to carding in that the fibers are combed. Thereafter the combed fibers are interlocked to form a web. Multiple webs can be overlapped to build up a desired weight. Random carding uses centrifugal force to throw fibers into a web with random orientation of the fibers. Again multilayers can be created to obtain the desired web weight. The dry laid components are then bonded together. Wet laid webs are made by a modified papermaking process in which the fibers are suspended in water, decanted on a screen, dried and bonded together.

The webs are bonded by a binding fiber such as low melt polymer fiber or bicomponent fiber as noted above. The web of fibers (binder fibers and absorbent) can be bonded together by thermal means. Thermal bonding melts the binder fibers in an oven (hot air, radiant or microwave), or heated calendar roll(s), or by ultrasonic energy. Next, the web is cooled thereby solidifying the melted binder fiber. The web now has sufficient rigid structure to be useful as a component of an absorbent pad.

The webs are made by merely mixing the binder fiber (either the low melt polymer fiber or bicomponent fiber, or both) with the absorbent fibers (with or without SAP) using dry laid or wet laid techniques. The absorbent is mixed with the binder fiber such that the binder fiber comprises from about 5 to about 25 percent by weight of the total web, with the remainder being substantially the absorbent. The web compositions of the present invention can be layered until their weight is in the range from about 20 to about 500 grams per square meter (gsm), preferably from about 50 to about 250 gsm. Thereafter, the web may be cut into various lengths and widths for end use applications, namely, fenestration drapes, dental bibs, eye pads, diapers, incontinent pads, sanitary napkins, wound dressing pads, air filters, liquid filters and fabrics such as drapes, bedding or pillows.

### TEST PROCEDURE

The dry strength of the web was measured according to TAPPItest method T 498 om-88. The web strength was tested on a 25.4x 203.2 millimeter strip for both the MD (machine direction) and CD (cross direction) with an Instron 1122 test machine. The tests were run at 127 mm original separation at a speed of 304.8 mm per minute. The strength is reported in units of g/25 mm.

Bonding Index is the square root of the product of the machine direction and cross direction strengths.

The dust test used a 127 x 127 mm section of the web, cut into 25.4 x 25.4 mm samples. The samples were put into a Fluff Fiberization machine. An air stream with 100 PSI was applied to the samples for 300 seconds. The loosed fiber (dust) was collected with a filter. The percent of weight lost was reported as the percent of dust.

### EXAMPLES

In the following examples various bicomponent fibers were made with a core of 0.55 IV PET and a sheath of various compositions. The bicomponent fibers comprised a 50/50 core/sheath with the sheath being mainly LLDPE. The LLDPE was obtained from Dow Chemical Company as Aspun XU 61800.34 (Dow 34), which contains 10% by weight incorporated MAH. Additives (tackifier, adhesion promoter and enhancement agent) in a preblend were mixed with the sheath polymer prior to fiber spinning. The tackifier was preblended with 40% concentrate of the sheath polymer. The bicomponent fibers, after being spun and drawn, were cut into 6mm lengths.

The webs comprised 12% bicomponent fiber by weight and 88% wood pulp. The pulp type employed was Waco 416. The percentage of tackifier, adhesion promoter, and enhancement agent used in the Examples (and set forth in the Tables) are based on the weight of the low melt base.

### Example 1

Various bicomponent fibers were as shown in Table 1. The adhesion promoters were maleic anhydride grafted polyethylene obtained from Dow Chemical as ASPUN XU 60769.07 (Dow07), ethylene-acrylic copolymers obtained from DuPont as BYNEL 2022 and from ExxonMobil as ESCOR AT-325. The tackifier was a glycerin ester of tall oil rosin obtained from Eastman Chemical as PERMLYN 2085.

Nonwoven webs were made from these bicomponent fibers with a wet-lay process to give a basis weight of 51 g/m². The web samples were dried at 100° C for 32 seconds and then bonded in a hot air oven at 135° C for 15 seconds. The bonding indices are shown in Table 1, and compared to the control which did not contain a tackifier.

**Table 1**

| Fiber | Adhesion Promoter, % | Tackifier, % | Bonding Temp., C | Bonding Index, g/25 mm | Relative to Control, % |
|---|---|---|---|---|---|
| Control | Dow 07, 10% | None | 135 | 250.9 | |
| 1 | Bynel 2022, 5% | Permalyn, 5% | 135 | 368.9 | 47.0 |
| 2 | Escor AT 325, 5% | Permalyn,5% | 135 | 285.4 | 13.8 |
| 3 | Dow 07, 5% | Permalyn, 5% | 135 | 388.1 | 54.7 |
| 4 | Escor AT 325, 8% | Pamalyn, 2% | 135 | 281.1 | 12.0 |

This example shows the improved tensile strength using a tackifier and adhesion promoter.

### Example 2

In this example wet laid webs were prepared in the same manner as in Example 1, and examined the effect on adhesion promoter and tackifier levels on web strength. The bicomponent compositions and bonding indices are reported in Table 2. The control was a sheath that contained no adhesion promoter or tackifier.

**Table 2**

| Fiber | Adhesion Promoter. % | Tackifier, % | Bonding Temp., C | Bonding Index, g/25 mm | Relative to Control, % |
|---|---|---|---|---|---|
| Control | None | None | 135 | 314.3 | |
| 5 | Dow 07,5% | None | 135 | 267.0 | -15.0 |
| 6 | Dow 07,10% | None | 135 | 339.7 | 8.1 |
| 7 | None | Permalyn, 5% | 135 | 415.7 | 32.3 |
| 8 | Dow 07, 5% | Permalyn,5% | 135 | 442.2 | 40.7 |
| 9 | Dow 07,10% | Permalyn, 5% | 135 | 412.5 | 31.2 |
| 10 | None | Permalyn, 10% | 135 | 422.3 | 34.4 |
| Control | None | None | 175 | 378.3 | |
| 5 | Dow 07. 5% | None | 175 | 345.7 | -8.6 |
| 6 | Dow 07, 10% | None | 175 | 401.6 | 6.2 |
| 7 | None | Permalyn, 5% | 175 | 405.7 | 7.2 |
| 8 | Dow 07, 5% | Permalyn, 5% | 175 | 493.4 | 30.4 |
| 9 | Dow 07, 10% | Permalyn, 5% | 175 | 492.9 | 30.3 |
| 10 | None | Permalyn, 10% | 175 | 444.3 | 17.4 |

This example shows that a tackifier alone, without an adhesion promoter, improves the bonding index of the web.

### Example 3

This example studies the effect of tackifier level using webs prepared as in Example 1. The bicomponent compositions and bonding indices are reported in Table 3. The control was a sheath that contained 5 % Dow 07 adhesion promoter.

**Table 3**

| Fiber | Adhesion Promoter, % | Tackifier, % | Bonding Temp., C | Bonding Index, g/25 mm | Relative to Control, % |
|---|---|---|---|---|---|
| Control | Dow 07, 5% | None | 135 | 210. I | |
| 11 | Dow 07, 5% | Permalyn 2085, 1% | 135 | 337.7 | 60.8 |
| 12 | Dow 07, 5% | Permalyn 2085, 2.5% | 135 | 346.3 | 64.8 |
| 13 | Dow 07,5% | Permalyn 2085,3.75% | 135 | 352.6 | 67.8 |
| 14 | Dow 07, 5% | Permalyn 2085, 5% | 135 | 401.6 | 91.2 |
| | | | | | |
| Control | Dow 07, 5% | None | 175 | 268.2 | |
| 11 | Dow 07, 5% | Permalyn 2085, 1% | 175 | 431.0 | 60.7 |
| 12 | Dow 07,5% | Permalyn 2085, 2.5% | 175 | 351.4 | 31.0 |
| 13 | Dow 07, 5% | Permalyn 2085, 3.75% | 175 | 456.1 | 70.1 |
| 14 | Dow 07, 5% | Permalyn 2085, 5% | 175 | 452.7 | 68.8 |

This example shows that even a low level of tackifier, 1 % by weight, improves the bonding index dramatically.

### Example 4

Bicomponent fibers were prepared as in Example 1. These fibers were air laid with the wood pulp to give webs with a basis weight of 175 g/m². The web passed through a dryer with 15 seconds residence time at 140 or 175° C. The bicomponent compositions and bonding indices are reported in Table 4. The control was a sheath that contained 10 % Dow 07 adhesion promoter. In this example an enhancement agent, TiO2, was used. The TiO2 was preblended with the sheath polyethylene (Dow 34) at a 35% concentration.

**Table 4**

| Fiber | Adhesion Promoter, % | Tackifier, % | TiO₂, % | Bonding Temp., C | Bonding Index, g/25mm | Relative to Control, % |
|---|---|---|---|---|---|---|
| Control | Dow 07,10% | None | None | 140 | 267.0 | |
| 15 | Dow 07,5% | Permalyn 2085, 2.5% | None | 140 | 342.4 | 28.2 |
| 16 | Dow 07,5% | Permalyn 2085, 2.5% | 0.70 | 140 | 414.9 | 55.4 |
| 17 | Dow 07,5% | Permalyn 2085,2.5% | 0.35 | 140 | 398.9 | 49.4 |
| 18 | Dow 07,5% | Permalyn 2085, 5% | 0.35 | 140 | 413.8 | 55.0 |
| 19 | Dow 07,5% | Permalyn 2085, 5% | 0.70 | 140 | 348.0 | 30.3 |

The enhancement agent improved the bonding index.
Dust formation in air-laid processes is of concern. The webs from the control and runs 16 and 19, bonded at 140° C were subjected to the dust test. The results are shown in Table 5.

**Table 5**

| Fiber | Adhesion Promoter, % | Tackifier, % | TiO₂, % | Bonding Temp., C | Dust, % | Dust reduction |
|---|---|---|---|---|---|---|
| Control | Dow 07, 10% | None | None | 140 | 7.95 | |
| 16 | Dow 07, 5% | Permalyn 2085, 2.5% | 0.7 | 140 | 6.45 | 18.9 |
| 19 | Dow 07, 5% | Permalyn 2085,5% | 0.7 | 140 | 6.96 | 12.5 |

The tackifier with enhancement agent reduced the dust formation.

## Claims

1. An improved binder fiber comprising the combination of a low melt polyethylene base and a tackifier comprised from 1 to 5 % by weight of said low melt polyethylene base, said low melt polyethylene base is low melt fiber, the low melting portion of bicomponent fiber, or both, wherein a nonwoven web made from such binder fiber has a bonding index at least 13.8% greater than a web containing said binder fiber without said tackifier.

2. The improved binder fiber-of claim 1, wherein said tackifier is selected from the class of rosin, rosin esters, terpene based, piperylene based, and hydrocarbon based compounds.

3. The improved binder fiber of claim 1, wherein said bicomponent fiber has a high melting portion.

4. The improved binder fiber of claim 3, wherein said high melting portion is selected from the class of polyamide, polyester, polyolefin, polyacrylate, and mixtures thereof.

5. The improved binder fiber of claim 4, wherein said high melting portion is polyester.

6. The improved binder fiber of claim 4, wherein said high melting portion is polyolefin.

7. The binder fiber of claim 3, wherein said low melting base comprises from about 5% to about 75 % by weight of said bicomponent fiber.

8. The improved binder fiber of claim 1, wherein said polyethylene is selected from the class of HDPE, MDPE, LDPE, LLDPE, ULDPE, or mixtures of these.

9. The improved binder fiber of claim 1, wherein said low melt polymer fiber consists essentially of said low melt base and said tackifier.

10. The improved binder fiber of claim 1, additionally comprising an adhesion promoter in said low melt base.

11. The improved binder fiber of claim 10, wherein said adhesion promoter is selected from the class of maleic acid or maleic anhydride grafted polyolefin, ethylene-acrylic copolymers, or a combination of these.

12. The improved binder fiber of claim 11, wherein said grafted polyolefin contains incorporated maleic acid or maleic anhydride in the range from about 0.05 to about 2.0 weight % of said low melt polyethylene base.

13. The improved binder fiber of claim 11, wherein said ethylene-acrylic copolymers are present in a range of about 1 to about 20 weight % of said low melt base.

14. The improved binder fiber of claim 1, additionally comprising an enhancement agent in said low melt base.

15. The improved binder fiber of claim 14, wherein said enhancement agent is selected from the class of titanium dioxide, talc, silica, alum, calcium carbonate, calcium oxide, and magnesium oxide.

16. The improved binder fiber of claim 14, wherein said enhancement agent is present in a range of about 0.1 to 1.0 weight % of said low melt base.

17. A nonwoven web comprising binder fiber and absorbent, said binder fiber containing a low melt polyethylene base and a tackifier comprised from I to 5 % by weight of said low melt polyethylene base, said low melt polyetyhlene base is low melt polymer fiber, the low melting component of bicomponent fiber, or both, wherein said nonwoven web made from such binder fiber has a bonding index at least 13.8 % greater than a web containing said binder fiber without said tackifier.

18. The web of claim 17, wherein said binder fiber is from about 5 to about 25 weight % of said web.

19. The web of claim 17, wherein said absorbent comprises natural absorbents, super absorbent polymer, or both.

20. The web of claim 17, wherein said bicomponent fiber has a high melting portion.

21. The web of claim 20, wherein said high melting portion is selected from the class of polyamides, polyesters, polyolefins, polyacrylates, and mixtures thereof.

22. The web of claim 21, wherein said high melting portion is polyester.

23. The web of claim 21, wherein said high melting portion is polyolefin.

24. The web of claim 17, wherein said tackifier is selected from the class of rosin, rosin esters, terpene based, piperylene based, and hydrocarbon based compounds.

25. The web of claim 17, wherein said low melt polymer fiber is substantially low melt base and said tackifier.

26. The web of claim 17, wherein said polyethylene is selected from the class of HDPE, MDPE, LDPE, LLDPE, ULDPE, or mixtures of these.

27. The web of claim 17, additionally comprising an adhesion promoter in said low melt base.

28. The web of claim 27, wherein said adhesion promoter is selected from the class of maleic acid or maleic anhydride grafted polyolefin, ethylene-acrylic copolymers, or a combination of these.

29. The web of claim 28, wherein said grafted polyolefin contains incorporated maleic acid or maleic anhydride in the range from about 0.05 to about 2.0 weight % of said low melt base.

30. The web of claim 28, wherein said ethylene-acrylic copolymers are present in a range of about 1 to about 20 weight % of said low melt base.

31. The web of claim 27, wherein said bicomponent fiber has a high melting portion.

32. The web of claim 31, wherein said high melting portion is selected from the class of polyamides, polyesters, polyolefins, polyacrylates, and mixtures thereof.

33. The web of claim 32, wherein said high melting portion is polyester.

34. The web of claim 32, wherein said high melting portion is polyolefin.

35. The web of claim 17, wherein said low melt base also contains enhancement agent.

36. The web of claim 35, wherein said enhancement agent is selected from the class of titanium dioxide, talc, silica, alum, calcium carbonate, calcium oxide, and magnesium oxide.

37. The web of claim 35, wherein said enhancement agent is present in a range from about 0.1 to 1.0 weight % of said low melt base.

## Patentansprüche

1. Verbesserte Bindefaser, umfassend die Kombination einer niedrigschmelzenden Polyethylenbasis und eines darauf bezogen 1 bis 5 Gew.-% ausmachenden Klebrigmachers, wobei es sich bei der niedrigschmelzenden Polyethylenbasis um eine niedrigschmelzende Faser, um den niedrigschmelzenden Anteil einer Bikomponentenfaser oder um beides handelt, bei der ein damit hergestellter Vliesstoff gegenüber einem die Bindefaser ohne den Klebrigmacher enthaltenden Vliesstoff einen um mindestens 13,8% größeren Verfestigungsindex aufweist.

2. Verbesserte Bindefaser nach Anspruch 1, bei der der Klebrigmacher ausgewählt ist aus der Klasse Kolophonium, Kolophoniumester, terpen-, piperylen- und kohlenwasserstoffbasierte Verbindungen.

3. Verbesserte Bindefaser nach Anspruch 1, bei der die Bikomponentenfaser über einen hochschmelzenden Anteil verfügt.

4. Verbesserte Bindefaser nach Anspruch 3, bei der der hochschmelzende Anteil ausgewählt ist aus der Klasse Polyamid, Polyester, Polyolefin, Polyacrylat und Mischungen davon.

5. Verbesserte Bindefaser nach Anspruch 4, bei der es sich bei dem hochschmelzenden Anteil um Polyester handelt.

6. Verbesserte Bindefaser nach Anspruch 4, bei der es sich bei dem hochschmelzenden Anteil um Polyolefin handelt.

7. Bindefaser nach Anspruch 3, bei der die niedrigschmelzende Basis etwa 5 bis etwa 75 Gew.-% der Bikomponentenfaser ausmacht.

8. Verbesserte Bindefaser nach Anspruch 1, bei der das Polyethylen ausgewählt ist aus der Klasse HDPE, MDPE, LDPE, LLDPE, ULDPE oder Mischungen davon.

9. Verbesserte Bindefaser nach Anspruch 1, bei der die niedrigschmelzende Polymerfaser im wesentlichen aus der niedrigschmelzenden Basis und dem Klebrigmacher besteht.

10. Verbesserte Bindefaser nach Anspruch 1, bei der in der niedrigschmelzenden Basis zusätzlich ein Haftvermittler enthalten ist.

11. Verbesserte Bindefaser nach Anspruch 10, bei der der Haftvermittler ausgewählt ist aus der Klasse maleinsäure- oder maleinsäureanhydridgepfropftes Polyolefin, Ethylenacrylcopolymere oder eine Kombination davon.

12. Verbesserte Bindefaser nach Anspruch 11, bei der das gepfropfte Polyolefin die Maleinsäure bzw. das Maleinsäureanhydrid bezogen auf die niedrigschmelzende Polyethylenbasis zu etwa 0,05 bis etwa 2,0 Gew.-% enthält.

13. Verbesserte Bindefaser nach Anspruch 11, bei der die Ethylenacrylcopolymere bezogen auf die niedrigschmelzende Basis zu etwa 1 bis etwa 20 Gew.-% enthalten sind.

14. Verbesserte Bindefaser nach Anspruch 1, bei der in der niedrigschmelzenden Basis zusätzlich ein Verstärkungsmittel enthalten ist.

15. Verbesserte Bindefaser nach Anspruch 14, bei der das Verstärkungsmittel ausgewählt ist aus der Klasse Titandioxid, Talk, Siliciumdioxid, Aluminiumoxid, Calciumcarbonat, Calciumoxid und Magnesiumoxid.

16. Verbesserte Bindefaser nach Anspruch 14, bei der das Verstärkungsmittel bezogen auf die niedrigschmelzende Basis zu etwa 0,1 bis 1,0 Gew.-% enthalten ist.

17. Vliesstoff mit Bindefaser und Absorber, wobei die Bindefaser eine niedrigschmelzende Polyethylenbasis und einen darauf bezogen 1 bis 5 Gew.-% ausmachenden Klebrigmacher umfaßt, wobei es sich bei der niedrigschmelzenden Polyethylenbasis um eine niedrigschmelzende Polymerfaser, um den niedrigschmelzenden Anteil einer Bikomponentenfaser oder um beides handelt, bei dem der mit einer solchen Bindefaser hergestellte Vliesstoff gegenüber einem die Bindefaser ohne den Klebrigmacher enthaltenden Vliesstoff einen um mindestens 13,8% größeren Verfestigungsindex aufweist.

18. Vliesstoff nach Anspruch 17, bei dem die Bindefaser etwa 5 bis etwa 25 Gew.-% des Vliesstoffs ausmacht.

19. Vliesstoff nach Anspruch 17, bei dem der Absorber natürliche Absorber, Superabsorber oder beides umfaßt.

20. Vliesstoff nach Anspruch 17, bei dem die Bikomponentenfaser über einen hochschmelzenden Anteil verfügt.

21. Vliesstoff nach Anspruch 20, bei dem der schwer schmelzende Anteil ausgewählt ist aus der Klasse Polyamide, Polyester, Polyolefine, Polyacrylate und Mischungen davon.

22. Vliesstoff nach Anspruch 21, bei dem es sich bei dem hochschmelzenden Anteil um Polyester handelt.

23. Vliesstoff nach Anspruch 21, bei dem es sich bei dem hochschmelzenden Anteil um Polyolefin handelt.

24. Vliesstoff nach Anspruch 17, bei dem der Klebrigmacher ausgewählt ist aus der Klasse Kolophonium, Kolophoniumester, terpen-, piperylen- und kohlenwasserstoffbasierte Verbindungen.

25. Vliesstoff nach Anspruch 17, bei dem es sich bei der niedrigschmelzenden Polymerfaser weitgehend um die niedrigschmelzende Basis und den Klebrigmacher handelt.

26. Vliesstoff nach Anspruch 17, bei dem das Polyethylen ausgewählt ist aus der Klasse HDPE, MDPE, LDPE, LLDPE, ULDPE oder Mischungen davon.

27. Vliesstoff nach Anspruch 17, bei dem in der niedrigschmelzenden Basis zusätzlich ein Haftvermittler enthalten ist.

28. Vliesstoff nach Anspruch 27, bei dem der Haftvermittler ausgewählt ist aus der Klasse maleinsäure- oder maleinsäureanhydridgepfropftes Polyolefin, Ethylenacrylcopolymere oder eine Kombination davon.

29. Vliesstoff nach Anspruch 28, bei dem das gepfropfte Polyolefin die Maleinsäure bzw. das Maleinsäureanhydrid bezogen auf die niedrigschmelzende Basis zu etwa 0,05 bis etwa 2,0 Gew.-% enthält.

30. Vliesstoff nach Anspruch 28, bei dem die Ethylenacrylcopolymere bezogen auf die niedrigschmelzende Basis zu etwa 1 bis etwa 20 Gew.-% enthalten sind.

31. Vliesstoff nach Anspruch 27, bei dem die Bikomponentenfaser über einen hochschmelzenden Anteil verfügt.

32. Vliesstoff nach Anspruch 31, bei dem der hochschmelzende Anteil ausgewählt ist aus der Klasse Polyamide, Polyester, Polyolefine, Polyacrylate und Mischungen davon.

33. Vliesstoff nach Anspruch 32, bei dem es sich bei dem hochschmelzenden Anteil um Polyester handelt.

34. Vliesstoff nach Anspruch 32, bei dem es sich bei dem hochschmelzenden Anteil um Polyolefin handelt.

35. Vliesstoff nach Anspruch 17, bei dem die leicht schmelzende Basis ferner ein Verstärkungsmittel enthält.

36. Vliesstoff nach Anspruch 35, bei dem das Verstärkungsmittel ausgewählt ist aus der Klasse Titandioxid, Talk, Siliciumdioxid, Aluminiumoxid, Calciumcarbonat, Calciumoxid und Magnesiumoxid.

37. Vliesstoff nach Anspruch 35, bei dem das Verstärkungsmittel bezogen auf die niedrigschmelzende Basis zu etwa 0,1 bis 1,0 Gew.-% enthalten ist.

## Revendications

1. Fibre liante améliorée comprenant l'association d'un composant de base de type polyéthylène à bas point de fusion et d'un adhésif, comprenant de 1 à 5 % en poids du dit composant de base de type polyéthylène à bas point de fusion, ledit composant de base de type polyéthylène à bas point de fusion étant une fibre à bas point de fusion, la partie à bas point de fusion d'une fibre bicomposant ou les deux, une nappe non tissée produite à partir d'une telle fibre liante ayant un indice de liaison d'au moins 13,8 % supérieur à celui d'une nappe contenant ladite fibre liante sans ledit adhésif.

2. La fibre liante améliorée de la revendication 1, dans laquelle ledit adhésif est choisi parmi la classe de la colophane, des esters de colophane, des composés dérivés de terpène, dérivés de pipérylène et dérivés d'hydrocarbure.

3. La fibre liante améliorée de la revendication 1, dans laquelle ladite fibre bicomposant ayant une partie à point de fusion élevé.

4. La fibre liante améliorée de la revendication 3, dans laquelle ladite partie à point de fusion élevé, est choisie parmi la classe des polyamides, des polyesters, des polyoléfines, des polyacrylates et les mélanges de ceux-ci.

5. La fibre liante améliorée de la revendication 4, dans laquelle ladite partie à point de fusion élevé consiste en un polyester.

6. La fibre liante améliorée de la revendication 4, dans laquelle ladite partie à point de fusion élevé consiste en une polyoléfine.

7. La fibre liante de la revendication 3, dans laquelle ledit composant de base à bas point de fusion comprend d'environ 5 % environ 75 % en poids de ladite fibre bicomposant.

8. La fibre liante améliorée de la revendication 1, dans laquelle ledit polyéthylène est choisi parmi la classe du polyéthylène haute densité (HDPE), du polyéthylène à moyenne densité (MDPE), du polyéthylène à basse densité (LDPE), du polyéthylène linéaire à base densité (LLDPE), du polyéthylène à très haute densité (ULDPE) ou les mélanges de ceux-ci.

9. La fibre liante améliorée de la revendication 1, dans laquelle ladite fibre de polymère à bas point de fusion consiste essentiellement en ledit composant de base à bas point de fusion et en ledit adhésif.

10. La fibre liante améliorée de la revendication 1, comprenant en outre un promoteur d'adhérence dans ledit composant de base à bas point de fusion.

11. La fibre liante améliorée de la revendication 10, dans laquelle ledit promoteur d'adhérence est choisi parmi la classe des polyoléfines greffées par l'acide maléique ou l'anhydride maléique, les copolymères d'acide acrylique et d'éthylène ou une association de ceux-ci.

12. La fibre liante améliorée de la revendication 11, dans laquelle ladite polyoléfine greffée incorpore de l'acide maléique ou de l'anhydride maléique dans la plage d'environ 0,05 à environ 2,0 % du poids du dit composant de base de type polyéthylène à bas point de fusion.

13. La fibre liante améliorée de la revendication 11, dans laquelle lesdits copolymères d'acide acrylique et d'éthylène sont présents dans une plage d'environ 1 à environ 20 % du poids du dit composant de base à bas point de fusion.

14. La fibre liante améliorée de la revendication 1, comprenant en outre un agent de renforcement dans ledit composant de base à bas point de fusion.

15. La fibre liante améliorée de la revendication 14, dans laquelle ledit agent de renforcement est choisi parmi la classe du dioxyde de titane, du talc, de la silice, de l'alun, du carbonate de calcium, de l'oxyde de calcium et de l'oxyde de magnésium.

16. La fibre liante améliorée de la revendication 14, dans laquelle ledit agent de renforcement est présent dans une plage d'environ 0,1 à 1,0 % du poids du dit composant de base à bas point de fusion.

17. Nappe non tissée comprenant une fibre liante et un absorbant, ladite fibre liante contenant un composant de base de type polyéthylène à bas point de fusion et un adhésif, comprenant de 1 à 5 % en poids du dit composant de base de type polyéthylène à bas point de fusion, ledit composant de base de type polyéthylène à bas point de fusion étant une fibre de polymère à bas point de fusion, le composant à bas point de fusion d'une fibre bicomposant, ou les deux, ladite nappe non tissée produite à partir d'une telle fibre liante ayant un indice de liaison d'au moins 13,8 % supérieur à celui d'une nappe contenant ladite fibre liante sans ledit adhésif.

18. La nappe de la revendication 17, dans laquelle ladite fibre liante représente environ 5 à environ 25 % du poids de ladite nappe.

19. La nappe de la revendication 17, dans laquelle ledit absorbant comprend des absorbants naturels, un polymère super absorbant ou les deux.

20. La nappe de la revendication 17, dans laquelle ladite fibre bicomposant a une partie à point de fusion élevé.

21. La nappe de la revendication 20, dans laquelle ladite partie à point de fusion élevé est choisie parmi la classe des polyamides, des polyesters, des polyoléfines, des polyacrylates et les mélanges de ceux-ci.

22. La nappe de la revendication 21, dans laquelle ladite partie à point de fusion élevé consiste en un polyester.

23. La nappe de la revendication 21, dans laquelle ladite partie à point de fusion élevé consiste en une polyoléfine.

24. La nappe de la revendication 17, dans laquelle ledit adhésif est choisi parmi la classe de la colophane, des esters de colophane, des composés dérivés de terpène, dérivés de pipérylène et dérivés d'hydrocarbure.

25. La nappe de la revendication 17, dans laquelle ladite fibre de polymère à bas point de fusion comprend principalement le composant de base à bas point de fusion et ledit adhésif.

26. La nappe de la revendication 17, dans laquelle ledit polyéthylène est choisi parmi la classe du HDPE, du MDPE, du LDPE, du LLDPE, du ULDPE ou les mélanges de ceux-ci.

27. La nappe de la revendication 17, comprenant en outre un promoteur d'adhérence dans ledit composant de base à bas point de fusion.

28. La nappe de la revendication 27, dans laquelle ledit promoteur d'adhérence est choisi parmi la classe des polyoléfines greffées par l'acide maléique ou l'anhydride maléique, des copolymères d'acide acrylique et d'éthylène ou une association de ceux-ci.

29. La nappe de la revendication 28, dans laquelle ladite polyoléfine greffée incorpore de l'acide maléique ou de l'anhydride maléique dans la plage d'environ 0,05 à environ 2,0 % du poids du dit composant de base à bas point de fusion.

30. La nappe de la revendication 28, dans laquelle lesdits copolymères d'acide acrylique et d'éthylène sont présents dans une plage d'environ 1 à environ 20 % du poids du dit composant de base à bas point de fusion.

31. La nappe de la revendication 27, dans laquelle ladite fibre bicomposant a une partie à point de fusion élevé.

32. La nappe de la revendication 31, dans laquelle ladite partie à point de fusion élevé est choisie parmi la classe des polyamides, des polyesters, des polyoléfines, des polyacrylates et les mélanges de ceux-ci.

33. La nappe de la revendication 32, dans laquelle ladite partie à point de fusion élevé consiste en un polyester.

34. La nappe de la revendication 32, dans laquelle ladite partie à point de fusion élevé consiste en une polyoléfine.

35. La nappe de la revendication 17, dans laquelle ledit composant de base à bas point de fusion comprend également un agent de renforcement.

36. La nappe de la revendication 35, dans laquelle ledit agent de renforcement est choisi parmi la classe du dioxyde de titane, du talc, de la silice, de l'alun, du carbonate de calcium, de l'oxyde de calcium et de l'oxyde de magnésium.

37. La nappe de la revendication 35, dans laquelle ledit agent de renforcement est présent dans une plage d'environ 0,1 à 1,0 % du poids du dit composant de base à bas point de fusion.
